

Patented Dec. 15, 1925.

1,566,239

## UNITED STATES PATENT OFFICE.

CHARLES E. SWETT, OF WEST ROXBURY, AND WILLARD E. SWIFT, OF WORCESTER, MASSACHUSETTS, ASSIGNEES TO UNITED STATES ENVELOPE COMPANY, OF SPRINGFIELD, MASSACHUSETTS, A CORPORATION OF MAINE.

## TREATMENT OF TRANSPARENT MATERIAL.

No Drawing.

Application filed August 31, 1923. Serial No. 580,442.

*To all whom it may concern:*

Be it known that we, CHARLES E. SWETT, a citizen of the United States, residing at West Roxbury, in the county of Suffolk and Commonwealth of Massachusetts, and WILLARD E. SWIFT, a citizen of the United States, residing at Worcester, in the county of Worcester and Commonwealth of Massachusetts, have invented a new and useful Improvement in the Treatment of Transparent Material, of which the following is a specification.

The present invention relates to the treatment of transparent material, for the purpose of reducing the glare, or reflection of light, from its surface. The invention is particularly applicable to the treatment of such material as is used for the transparent patches or panels of so-called window envelopes,— i. e., the type of envelope having an opening therein, over which is cemented a covering of glassine paper, or other similar transparent or semi-transparent material.

In window envelopes as thus manufactured, a troublesome feature is the glare or reflection of light from the surface of the patch or panel, this giving rise to objection on the part of those required to handle numbers of such envelopes, as for instance in the sorting of mail, particularly when the light falls at a small angle from the plane of the surface. The reduction or elimination of this glare, without substantial sacrifice of the transparency of the patch or panel, is the primary object of the present invention, the same involving a mode of treatment for the surface of the glassine paper, or other similar material, which leaves said surface in a substantially matt or non-glare condition.

This treatment, as contemplated by the present invention, consists, generally, in subjecting the surface of the panel material to frictional or rubbing action in the presence of a suitable lubricant; in this way, the character of the surface is so altered, in some degree presumably by the lifting or disarrangement of its fibres, that the glare therefrom is materially reduced, without impairment however of the visibility or light transmitting properties of the material. In carrying out the process, the lubricant may be applied either to the

material or to the device by which the rubbing or friction is produced; and we have discovered that a suitable and desirable lubricant, for the purpose described, consists of a mixture of sulphonated oil and water, with or without the addition of glycerine, or a mixture of alcohol, water and acetate of potash or soda. We have also discovered that the presence of some water in the composition of whatever lubricant is used is quite desirable, since water tends to soften the fibres of the material and thereby promotes any change in the fibrous structure which may take place. On the other hand, the presence of too much water in the lubricant is undesirable, on account of the tendency of the material to warp and cockle when wet.

When subjected as above described to lubricated frictional treatment, the surface of the material is left in a matt and substantially glareless condition, even after all traces of the lubricating substances have been washed off,— a circumstance which renders the material thus treated especially adapted to the manufacture of window envelopes, since said condition is attained in the absence of any glare-deadening deposit, such as might tend to flake off or become bruised when subjected to handling in a window envelope machine.

Our invention resides in the mode of treatment above described, by which the material is subjected to frictional or rubbing action in the presence of a suitable lubricant; it is obvious that lubricating mixtures other than those above described may be employed in a manner the same or similar to that above described, and we do not limit ourselves to the use of said specified substances or materials, except as set forth in certain of the appended claims.

We claim:

1. The herein described process of treating transparent panel material, which consists in subjecting the surface of said material to lubricated friction.
2. In the production of a matt or substantially glareless surface for transparent panel material, the improvement which consists in frictionally rubbing the material in the presence of a lubricant.
3. In the production of a matt or substantially glareless surface for transparent

panel material, the improvement which consists in frictionally rubbing the material in the presence of a lubricant containing a limited quantity of water.

5. 4. In the production of a matt or substantially glareless surface for transparent panel material, the improvement which consists in frictionally rubbing the material with an aqueous mixture which has a 10 softening action on the fibers of said material.

5. In the production of a matt or substantially glareless surface for transparent

panel material, the improvement which consists in frictionally rubbing the material in 15 the presence of a lubricant containing sulphonated oil.

6. In the production of a matt or substantially glareless surface for transparent panel material, the improvement which consists in frictionally rubbing the material with a mixture containing water and sulphonated oil. 20

CHARLES E. SWETT.  
WILLARD E. SWIFT.